

## UNITED STATES PATENT OFFICE

2,347,024

IMPREGNATING COMPOSITION FOR  
TEXTILE MATERIALS

Leo Beer, Philadelphia, Pa.

No Drawing. Application April 24, 1943,  
Serial No. 484,462

13 Claims. (Cl. 260—29)

This invention relates to a method and means for treating textile materials and has particular relation to a process and a composition for reducing or eliminating the tendency of textile materials to shrink in laundering, and simultaneously improving the wearing qualities of said materials.

The main object of my present invention consists in treating textile materials with a composition adapted to yield shrinkproof products of improved wearing quality.

Another object of my invention is to reduce or eliminate the tendency of textile materials to shrink, by means of impregnating solutions of relatively low concentration.

A further object of this invention consists in the use of impregnating solutions which reduce the tendency of textile materials to shrink without impairing other properties of said materials.

Further objects and the advantages of the present invention will be apparent to those skilled in the art from the following specification and the appended claims.

It has been known in the art to produce shrinkproof textile materials by introducing thermosetting formaldehyde condensation products, particularly condensation products of the urea-formaldehyde type into the textile materials and converting said condensation products into resinous substances by heating. It has been found, however, that these condensation products must be used for the treatment of textiles in solutions of relatively high concentrations in order to obtain shrinkproof effects. Furthermore, incorporation of the condensation products in the textile fibers in the corresponding, relatively high amounts, results in deterioration of the wearing properties of the treated materials, particularly their resistance to abrasion. It has been suggested, therefore, to improve the wearing properties of fibers containing urea-formaldehyde resins by the application of rubber latex in mixture with said resins (U. S. Patent No. 2,299,786 of Oct. 27, 1942).

I have now found that the necessity of using urea-formaldehyde type condensation products in relatively concentrated solutions, and the adherent disadvantage of adversely affecting certain properties of the textile material treated, can be avoided by the use of solutions containing low amounts of heat-hardenable urea-formaldehyde type condensation products in mixture with octadecyl-oxymethyl-pyridinium chloride, with or without the addition of a catalyst, as specified in the following examples.

In carrying out my present invention, the textile material to be treated is impregnated at ordinary room temperature by causing it to pass through an aqueous liquid containing the above described mixture of urea-formaldehyde or urea-thiourea-formaldehyde condensation product and octadecyl-oxymethyl-pyridinium chloride. In the preferred form of my invention, I use an aqueous solution containing about 2% by weight of the urea-formaldehyde type condensation product and about 0.3-0.6% of octadecyl-oxymethyl-pyridinium chloride. In the treatment of cellulosic materials it is advisable to add to the impregnating solution a small amount of a salt of a strong inorganic base, such as sodium or potassium, and a weak organic acid such as formic, acetic or lactic acid or an acid of similar strength. After passing through the impregnating solution, the textile material is squeezed out until it contains about 100% by weight of solution based on the weight of the dry starting material. The impregnated material is then dried at a relatively low temperature, f. e. at about 40°-70° C., preferably at 60°-70° C., and after drying heated for some minutes, f. e. 5-10 minutes, at 120-130° C. The impregnating solution may preferably contain a catalyst. I have found that the use of a catalyst consisting of about equal parts of hexamethylenetetramine and a suitable ammonium salt, such as ammonium sulfate, is advantageous, particularly in the treatment of cellulosic materials.

It has been found that textile materials, such as fabrics, spun goods, filaments, webs, etc. consisting of wool, natural or regenerated cellulose, cellulose derivatives, such as cellulose acetate, or mixtures of these materials may be successfully treated according to the present invention. The treated textile materials are shrinkproof and they show a substantial improvement with respect to their wearing qualities and particularly their resistance to abrasion. In the case of woolen materials the tendency to felt formation is also reduced.

*Example 1.*—Woolen stockings are wetted and immersed in an aqueous liquid containing in solution 2% by weight of a water-soluble urea-formaldehyde condensation product and 0.6% of octadecyl-oxymethyl-pyridinium chloride. The stockings are then squeezed or subjected to centrifugal action until they contain 100% by weight of liquid based on the dry weight of the starting material. They are then dried at about 60°-70° C. and finally heated for about 5 minutes at 120°-130° C. in a chamber heated by means of

hot air. If the product thus obtained is subjected to washing with an aqueous soap solution, it substantially retains its original shape and dimensions. The resistance to abrasion of the material treated shows a very substantial increase in comparison to that of the untreated material. While the latter is rubbed through at 1000 cycles in Taber's testing machine, the treated material requires 4000 cycles for obtaining the same effect under otherwise equal conditions.

*Example II.*—A fabric consisting of 50% wool and 50% of cotton is treated with an aqueous liquid containing in 1 liter of the solution

|                                                     | Grams |
|-----------------------------------------------------|-------|
| Urea - thiourea - formaldehyde condensation product | 18    |
| Octadecyl-oxymethyl-pyridinium chloride             | 6     |
| Sodium formate                                      | 1     |

The treatment of the fabric with the liquid, and the subsequent drying and heating are carried out in the manner described in Example I. The product is shrink-proof and is rubbed through at 1500 cycles in Taber's testing machine, in comparison to 800 cycles in the case of the untreated material.

*Example III.*—Rayon fabric consisting of viscose rayon warp and filling is treated with an aqueous liquid containing dissolved in 1 liter of water

|                                         | Grams |
|-----------------------------------------|-------|
| Urea-formaldehyde condensation product  | 22    |
| Octadecyl-oxymethyl-pyridinium chloride | 3     |
| Sodium formate                          | 0.5   |

The treatment of the fabric with liquid and the subsequent drying and heating are carried out substantially in the manner described in Example I. The product obtained shows an improvement of the resistance to abrasion of 500 cycles on Taber's testing device in comparison to 350 cycles in the case of the untreated starting material.

*Example IV.*—A cotton fabric consisting of cotton yarn in warp and filling is impregnated at 18°-20° C. with a solution of

|                                                     | Grams |
|-----------------------------------------------------|-------|
| Urea - thiourea - formaldehyde condensation product | 20    |
| Octadecyl-oxymethyl-pyridinium chloride             | 4     |
| Sodium formate                                      | 0.6   |
| Hexamethylene tetramine                             | 0.4   |
| Ammonium sulfate                                    | 0.4   |

in 1 liter of water. The treatment of the fabric is in all respects identical with that described in Example I. The product obtained is rubbed through at 850 cycles on the Taber machine in comparison to 600 cycles in the case of the untreated material.

*Example V.*—A fabric consisting of 50% of cotton and 50% of viscose rayon is treated in the manner described in Example I with the following solution:

|                                         | Grams |
|-----------------------------------------|-------|
| Urea-formaldehyde condensation product  | 20    |
| Octadecyl-oxymethyl-pyridinium chloride | 3     |
| Hexamethylene tetramine                 | 0.35  |
| Ammonium sulfate                        | 0.4   |
| Sodium lactate                          | 1     |

dissolved in 1 liter of water. Drying and heating of the impregnated fabric are also carried out in the manner described in Example I. The finished product is rubbed through at 600 cycles in the Taber machine in comparison to 450 cycles in the case of the untreated starting material.

The effect obtained in carrying out my present invention is unobvious because the use of an urea-formaldehyde type resin by itself under otherwise similar conditions does not result in a shrink-proof product, and because it could not be expected that deterioration of the textile product by the urea-formaldehyde compounds can be prevented by the presence of the octadecyl-oxymethyl-pyridinium chloride. Moreover, the use of said resin by itself causes deterioration of properties of the starting material while the combined use of resin and pyridinium salt under the conditions of my present invention, results in an improvement of said properties.

For example, a rayon fabric, which, in its original, untreated condition, is rubbed through in Taber's testing device at 400 cycles, requires only 250 cycles after being treated in the customary manner with urea-formaldehyde type condensation products. If, however, the same fabric is treated in accordance with the present invention with a mixture of urea-formaldehyde type condensation products and octadecyl-oxymethyl-pyridinium chloride, it will be rubbed through in Taber's testing device at 550 cycles.

The urea condensation products used in carrying out my present invention are prepared in a manner known per se, f. e. by condensing one mol of urea or a mixture of urea and thiourea, with 2 mols of formaldehyde to a water-soluble condensation product which is recovered from the aqueous solution. The figures stated in the above examples relate to the solid, technically pure condensation products.

It will be understood that this invention is not limited to the specific embodiments set forth in the above examples, and the details set forth in these examples, such as the amount of the ingredients used or their relative proportions etc., may be varied without departing from the spirit of the invention as defined in the appended claims.

I claim:

1. An impregnating composition for textile materials, said composition containing in aqueous solution about 0.3-0.6% by weight of octadecyl-oxymethyl-pyridinium chloride and about 1.8-2.2% by weight of a thermosetting condensation product selected from the group consisting of urea-formaldehyde and urea-thiourea-formaldehyde condensation products.

2. An impregnating composition for textile materials, said composition containing in aqueous solution about 0.3-0.6% by weight of octadecyl-oxymethyl-pyridinium chloride and about 1.8-2.2% by weight of a thermosetting condensation product selected from the group consisting of urea-formaldehyde and urea-thiourea-formaldehyde condensation products and a catalyst consisting of about equal parts of hexamethylene tetramine and ammonium sulfate.

3. An impregnating composition for textile materials, said composition containing in aqueous solution about 0.3-0.6% by weight of octadecyl-oxymethyl-pyridinium chloride and about 1.8-2.2% by weight of a thermo-setting urea-thiourea-formaldehyde condensation product.

4. An impregnating composition for textile materials, said composition containing in aqueous solution about 0.3-0.6% by weight of octadecyl-oxymethyl-pyridinium chloride and about 1.8-2.2% by weight of a thermo-setting urea-thiourea-formaldehyde condensation product, and a catalyst consisting of about equal parts of

hexamethylene tetramine and ammonium sulfate.

5. An impregnating composition for textile materials, said composition containing in aqueous solution about 0.3-0.6% by weight of octadecyl-oxymethyl-pyridinium chloride and about 1.8-2.2% by weight of a thermo-setting urea-formaldehyde condensation product.

6. An impregnating composition for textile materials, said composition consisting of 3-6 parts by weight of octadecyl-oxymethyl-pyridinium chloride and about 18-22 parts by weight of a thermo-setting urea-formaldehyde condensation product dissolved in one liter of water.

7. An impregnating composition for textile materials, said composition containing in aqueous solution about 0.3-0.6% by weight of octadecyl-oxymethyl-pyridinium chloride and about 1.8-2.2% by weight of a thermo-setting urea-formaldehyde condensation product and a catalyst consisting of about equal parts of hexamethylene tetramine and ammonium sulfate.

8. An impregnating composition for textile materials said composition containing in aqueous solution about 0.3-0.6% by weight of octadecyl-oxymethyl-pyridinium chloride and about 1.8-2.2% by weight of a thermo-setting condensation product selected from the group consisting of urea-formaldehyde and urea-thiourea-formaldehyde condensation products, and an alkali salt of a weak organic acid.

9. An impregnating composition for textile materials, said composition consisting of an aqueous solution containing about 2% by weight of a thermosetting condensation product selected from the group consisting of urea-formaldehyde and urea-thiourea-formaldehyde condensation products, and about 0.3-0.6% by weight of octadecyl-oxymethyl-pyridinium chloride.

10. An impregnating composition for textile materials, said composition consisting of an aqueous solution containing about 2% by weight of a thermosetting condensation product selected from the group consisting of urea-formaldehyde

and urea thiourea-formaldehyde condensation products, about 0.3-0.6% by weight of octadecyl-oxymethyl-pyridinium chloride, and about 0.05-0.1% by weight of an alkali salt of a weak organic acid.

11. An impregnating composition for textile materials, said composition consisting of an aqueous solution containing about 2% by weight of a thermosetting condensation product selected from the group consisting of urea-formaldehyde and urea-thiourea-formaldehyde condensation products, about 0.3-0.6% by weight of octadecyl-oxymethyl-pyridinium chloride, and about 0.05-0.1% by weight of an alkali salt of a weak organic acid, and a catalyst consisting of about equal parts of hexamethylene tetramine and ammonium sulfate.

12. A process for the treatment of textile materials, said process consisting in impregnating the textile material with an aqueous solution containing about 2% by weight of a thermosetting condensation product selected from the group consisting of urea-formaldehyde and urea-thiourea-formaldehyde condensation products and about 0.3-0.6% by weight of octadecyl-oxymethyl-pyridinium chloride, drying the impregnated material at a temperature below 70° C. and heating the dried material at 120°-130° C.

13. A process for the treatment of textile materials, said process consisting in introducing into the textile material 100% by weight of an aqueous solution containing about 2% by weight of a thermosetting condensation product selected from the group consisting of urea-formaldehyde and urea-thiourea-formaldehyde condensation products, about 0.3-0.6% by weight of octadecyl-oxymethyl-pyridinium chloride, about 0.05-0.1% by weight of an alkali salt of a weak organic acid, and a catalyst consisting of about equal parts of hexamethylene tetramine and ammonium sulfate, drying the impregnated material at 60°-70° C. and heating the dried material at 120°-130° C. for 5-10 minutes.

LEO BEER.